

## UNITED STATES PATENT OFFICE.

GEORGE CLIFTON DEETER, OF YORK, PENNSYLVANIA.

## METAL ALLOY.

No Drawing.

Application filed April 20, 1926. Serial No. 103,388.

My invention appertains generally to new and useful improvements in metal alloys and more particularly to an improved metal alloy for use in preparing or melting down 5 certain metals or combination of metals.

The primary object of my invention is the production of a metal alloy intended primarily for use as a deoxidizing and fluxing agent in the preparation or melting down of 10 certain metals or combination of metals.

Another very important object of my invention is the production of an improved metal alloy which will also act as a scavenger or cleanser, and by the use of which it is 15 possible to produce metals of maximum strength, density and ductility.

A further object of my invention is the production of such a metal alloy composed of a plurality of ingredients, all of which 20 may be readily obtained and which ingredients can be easily compounded.

My composition consists generally of a mixture of nickel, tin, manganese, phosphorus and copper.

In preparing my composition, I prefer to use the above ingredients in about the following proportions viz:

Nickel, 5% to 10%; tin, 3% to 10%; manganese, 75/100% to 5%; phosphorus, 30 25/100% to 3%; copper—the amount of copper used being the amount necessary to form 100%.

As seen from the above, the proportions of the ingredients can be somewhat varied as

may be found desirable but in the preferred 35 compounding of the alloy, the ingredients are preferably used in the following proportions and these proportions may be properly called the standard proportions.

Copper, 84%; nickel, 10%; tin, 5%; manganese, 75/100%; phosphorus, 25/100%.

My alloy may be used in varying percentages as an addition to other metals for accomplishing the objects enumerated hereinabove or it may be used as a whole to produce 45 castings for various purposes.

By the use of my improved alloy, it is possible, by the use of very small percentages, to obtain a superior casting with a dense fine 50 grain, increased tensile strength and improved machining qualities.

My alloy is used to great advantage in red and yellow brass and in low lead bronzes as a deoxidizer and strengthener and to further improve the machining and wearing 55 qualities thereof.

What I claim is:

1. A scavenging alloy consisting of the following metals taken in the proportions covering the following ranges; nickel, from 5 to 10%; tin, from 3 to 10%; manganese, from 75/100 to 5%; phosphorus from 25/100 to 3%; and copper from 72 to 92%.

2. A scavenging alloy consisting of 84% copper, 10% nickel, 5% tin, 75/100% manganese, and 25/100% phosphorus.

In testimony whereof I affix my signature.

GEORGE CLIFTON DEETER.